

[54] **METHOD FOR MANUFACTURING AN IMAGE PICKUP TUBE**

29/472.7; 316/17, 18, 19, 20; 317/235 NA;  
220/2.1 R, 2.1 A, 2.3; 357/6

[75] Inventors: **Shoichi Miyashiro, Yokohama; Shunji Shirouzu, Ayase; Kazuo Shimizu; Okio Yoshida, both of Yokohama, all of Japan**

[73] Assignee: **Tokyo Shibaura Electric Co., Ltd., Kawasaki, Japan**

[22] Filed: **Oct. 18, 1973**

[21] Appl. No.: **407,579**

**Related U.S. Application Data**

[60] Continuation-in-part of Ser. No. 329,576, Feb. 5, 1973, abandoned, which is a division of Ser. No. 105,823, Jan. 12, 1971, abandoned.

[30] **Foreign Application Priority Data**

Jan. 16, 1970 Japan..... 45-3798  
July 28, 1970 Japan..... 45-65546

[52] **U.S. Cl.**..... 316/19; 357/6

[51] **Int. Cl.<sup>2</sup>**..... H01J 9/18

[58] **Field of Search**..... 29/25.13, 25.14, 25.15,

[56]

**References Cited**

**UNITED STATES PATENTS**

|           |         |                     |            |
|-----------|---------|---------------------|------------|
| 3,253,331 | 5/1966  | Limansky.....       | 29/472.7   |
| 3,331,998 | 7/1967  | Zuleeg .....        | 317/235 NA |
| 3,419,746 | 12/1968 | Crowell et al.....  | 317/235 NA |
| 3,574,143 | 4/1971  | Vratny .....        | 317/235 NA |
| 3,664,895 | 5/1972  | Schaefer et al..... | 317/235 NA |
| 3,747,173 | 7/1973  | Lind.....           | 29/25.13   |

*Primary Examiner*—Roy Lake

*Assistant Examiner*—James W. Davie

*Attorney, Agent, or Firm*—Flynn & Frishauf

[57] **ABSTRACT**

An image pickup tube is manufactured by setting a PN junction type semiconductor target having a resistive sea made of cadmium telluride in a glass envelope and heating the envelope at 120°C to 400°C to effect evacuation.

**4 Claims, 4 Drawing Figures**



FIG. 1



FIG. 2



FIG. 4



FIG. 3



## METHOD FOR MANUFACTURING AN IMAGE PICKUP TUBE

### CROSS-REFERENCE TO RELATED APPLICATION

This is Continuation-in-part of U.S. Pat. application Ser. No. 329,576, filed on Feb. 5 1973, now abandoned, which in turn is a Division of U.S. Pat. application Ser. No. 105,823, filed Jan. 12, 1971, now abandoned.

### BACKGROUND OF THE INVENTION

This invention relates to a method for manufacturing an image pickup tube having a semiconductor target with a plurality of PN junctions.

An image pickup tube such as a vidicon and electron multiplication type camera tube generally includes a semiconductor target to convert photoimage signals to electric image signals. Such target comprises an N-type silicon substrate and a plurality of island regions arranged on that side of the substrate which is scanned by electron beams emitted from an electron gun. That surface of the substrate subjected to scanning is coated, to the exclusion of the island regions, with a protective layer made of insulating material, for example, silicon dioxide. Further on the protective layer is formed a semi-insulating layer having a discharge time constant longer than one frame period of television scanning and shorter than the discharge time constant of the insulating layer, thereby enabling any charge on the film to leak sidewise so as to prevent the film from being unnecessarily charged when it is exposed to light. Such a semi-insulating layer is usually made of antimony triselenide or antimony trisulfide. When an envelope containing a semiconductor target formed of such substance is heated to be more evacuated, then the semiconductor layer has its resistivity prominently varied by said heat treatment, failing to present desired characteristics relative to, for example, dark current and resolution. Furthermore, when heated to above 350°C the above-mentioned substance is revolatilized to be rendered unusable and found inadapted to be applied to an image pickup tube, for example, an electron multiplication type camera tube, whose photoelectric surface requires high temperature treatment.

In view of the problem involved in the heat treatment, it may be contemplated to prepare the semi-insulating layer from cadmium selenide or cadmium sulfide. However, each substance has a relatively low resistivity of about  $10^{-8}$  to  $10^{-10}$   $\Omega\text{-cm}^{-2}$  and indicates too low a resolution capacity for practical application.

When the insulating layer is formed from the above-mentioned material, its resistivity is greatly changed due to a slight change in evaporation conditions and, therefore, difficulty is presented in obtaining image pickup tubes having substantially equal characteristics, thus resulting in a poor yield.

### SUMMARY OF THE INVENTION

It is accordingly the object of this invention to provide a method for manufacturing an image pickup tube equipped with a semiconductor target having a semi-insulating layer less liable to be changed in its characteristics even on heat treatment.

In an aspect of this invention there is provided a method for manufacturing an image pickup tube comprising the steps of preparing a semiconductor target including a semiconductor substrate of one conductiv-

ity type, a plurality of island regions of the opposite type formed on one side of the substrate, an insulating layer coated on said one side of the substrate to the exclusion of the island regions thereof, and a semi-insulating layer of cadmium telluride coated at least on the insulating layer; introducing the semiconductor target into a glass envelope; and evacuating the glass envelope while heating it in a range of 120° to 400°C.

The semiconductor layer made of cadmium telluride has a resistivity of the order of  $10^{12}$   $\Omega\text{-cm}^{-2}$  at room temperature. The resistivity of the semiconductor layer is gradually increased with heating temperature and when the heating temperature reaches about 120°C, then the resistivity of the semiconductor layer is decreased. Even when about 400°C, a limit of the heat treatment of the image pickup tube, is attained, the layer still has a resistivity close to  $10^{12}$   $\Omega\text{-cm}^{-2}$ . Consequently, the image pickup tube according to this invention is satisfied in its resolution independently of the heat treatment.

It is commonly required to heat a semiconductor target at a temperature of 400°C for 60 minutes in an  $\text{H}_2$  atmosphere before the formation of a semi-insulating layer. This heat treatment is intended to correct the state of boundary between the semiconductor substrate and the insulating layer to prevent a current leakage along the boundary which would cause resolution to be reduced. Generally, an envelope is formed from a glass having a softening point of about 400°C. Use of glass having a softening point of above 400°C makes it difficult to, for example, partially fuse or bore an envelope in an attempt to fixedly attach metal leads and sealing metal ring to the envelope. On the other hand, when use is made of glass having a softening point of below 400°C, an envelope causes deformation or damage during heat treatment, since it is lower than the temperature at which the envelope is heat treated.

It is preferred that the lower limit of the aforementioned heat treatment be about 120°C at which a best resolution is attained i.e. a highest resistivity of the cadmium telluride layer is attained. With a temperature close to 120°C there is no fear that an indium seal will be melted by heat treatment. When the temperature of heat treatment is prominently raised from this lower temperature limit so as to improve a getter effect, then it is preferred that an aluminum seal be used, since the indium seal may be melted. Where attention is paid only to the getter effect, it is preferable that heat treatment be of the order of 250°C.

### BRIEF DESCRIPTION OF THE DRAWING

FIG. 1 is a cross section of a vidicon as manufactured according to this invention;

FIG. 2 is a cross section of an electron multiplication tube according to this invention;

FIGS. 3 and 4 are cross sections showing different semiconductor target as used in the above-mentioned image pickup tube.

### DESCRIPTION OF THE PREFERRED EMBODIMENT

There will now be described, by reference to accompanying drawings, a method for manufacturing an image pickup tube, especially a vidicon.

Referring to FIG. 3 there is shown a semiconductor target 7 as used in a vidicon. A reference numeral 1 denotes an N-type silicon substrate about 20 microns thick. On one side of the substrate 1 are provided in a

matrix arrangement a plurality of a P-type island regions 2 which, together with the substrate, define PN junctions therebetween. The island regions 2 are formed by diffusing boron in the substrate 1 so as to have a diameter of, for example, 6 microns and be spaced from each other at a pitch of 15 microns. On the aforementioned side of the substrate 1 including the exposed parts of the PN junctions excluding the island regions 2 is formed an insulating layer 3 of silicon dioxide about 0.5 micron thick. This insulating layer may be constituted by the silicon dioxide layer as it is which is used as making material in forming the island regions. Of course, use may be made of an insulating layer made of other material, for example, silicon monoxide or silicon nitride. The substrate 1 coated with the insulating layer 3 is heated at 400°C for 60 minutes in an H<sub>2</sub> atmosphere to decrease the charge density of the surface of the substrate so that a surface current flowing in the boundary area between the substrate and insulating layer may be effectively decreased. On the aforementioned side of the substrate is coated a semi-insulating layer 4 of cadmium telluride about 500 Å thick so as to cover all the insulating layer 3 and island regions 2. Said cadmium telluride layer 4 may be formed by the ordinary film depositing technique, for example, a vacuum evaporation process. The periphery of the opposite side of the substrate 1 is formed thick to increase its mechanical strength. On said side is formed an N<sup>+</sup> type layer 5. An aluminum electrode 6 is deposited on the peripheral portion of the N<sup>+</sup> type layer 5.

The modified semiconductor target shown in FIG. 4 is only different from the preceding one in that the semi-insulating layer 4 covers the protective insulating

seal (i.e., of the type shown in U.S. Pat. No. 2,876,596 Kessler, Jr.) is used instead of the indium seal, it is possible to heat treat the envelope at higher temperature ranging 250°C to 400°C.

The vidicon so manufactured is characterized in that it is sufficiently practicable in respect of dark current, resolution etc., since the resistive sea of the semiconductor target is made of cadmium telluride and the envelope is heated at to least 120°C during the evacuation.

An electron multiplication tube as shown in FIG. 2 is constituted by an image section 10a and a scanning section 10b. Since the scanning section has substantially the same construction as that of the vidicon, its explanation is omitted and only the image section will be described.

The forward section or image section 10a of the envelope 10 includes a photosensitive surface 17 for emitting electrons according to an incident light, and an electrode 18 for accelerating emitted electrons to conduct them to the semiconductor target 7.

Where the metal seal 16' of the electron multiplication tube is made of aluminum, the envelope can be heat treated at about 250°C.

For reference, Table 1 shows changes in physical properties involved in the heat treatment of a prior art semiconductor target including a semi-insulating layer formed of antimony triselenide (Sb<sub>2</sub>Se<sub>3</sub>), antimony trisulfide (Sb<sub>2</sub>S<sub>3</sub>), cadmium selenide (CdSe) and cadmium sulfide (CdS) respectively, in comparison with those of a semiconductor target whose insulating layer is made of cadmium telluride according to this invention.

Table 1

| Component                       | Without heat treatment                             | Treated in vacuum for 3 hrs. at 120°C | Treated in vacuum for 3 hrs. at 250°C                              | Treated in vacuum for 3 hrs. at 350°C              | Treated in vacuum for 3 hrs. at 400°C              |
|---------------------------------|----------------------------------------------------|---------------------------------------|--------------------------------------------------------------------|----------------------------------------------------|----------------------------------------------------|
| Sb <sub>2</sub> Se <sub>3</sub> | $1.7 \times 10^{11}$ $\Omega \cdot \text{cm}^{-2}$ | Same as left                          | $3.3 \times 10^{11}$ $\Omega \cdot \text{cm}^{-2}$<br>(Solidified) | Revoltalized                                       | Revoltalized                                       |
| Sb <sub>2</sub> S <sub>3</sub>  | $1.8 \times 10^{12}$ $\Omega \cdot \text{cm}^{-2}$ | "                                     | $4.4 \times 10^{13}$ $\Omega \cdot \text{cm}^{-2}$<br>(Solidified) | "                                                  | "                                                  |
| CdTe                            | $2.2 \times 10^{12}$ $\Omega \cdot \text{cm}^{-2}$ | "                                     | $5.3 \times 10^{12}$ $\Omega \cdot \text{cm}^{-2}$                 | $3.8 \times 10^{12}$ $\Omega \cdot \text{cm}^{-2}$ | $6.0 \times 10^{11}$ $\Omega \cdot \text{cm}^{-2}$ |
| CdSe                            | $7.2 \times 10^9$ $\Omega \cdot \text{cm}^{-2}$    | "                                     | $9.4 \times 10^9$ $\Omega \cdot \text{cm}^{-2}$                    | $8.6 \times 10^9$ $\Omega \cdot \text{cm}^{-2}$    | $4.5 \times 10^8$ $\Omega \cdot \text{cm}^{-2}$    |
| CdS                             | $6.5 \times 10^{10}$ $\Omega \cdot \text{cm}^{-2}$ | "                                     | $8.2 \times 10^{10}$ $\Omega \cdot \text{cm}^{-2}$                 | $7.5 \times 10^{10}$ $\Omega \cdot \text{cm}^{-2}$ | $3.7 \times 10^9$ $\Omega \cdot \text{cm}^{-2}$    |

layer 3 alone and is not deposited on the P-type island regions.

Reference is invited to FIG. 1. An envelope 10 made of glass having a softening point of about 400°C is prepared, and a mesh electrode 11, accelerating electrode 12 and electron gun 13 are mounted in the envelope by a known manner. The aforesaid semiconductor target 7 is mounted through a transparent electrode 14 to a face plate 15 in a manner to permit the electrode 6 of the semiconductor target to be brought into contact with the transparent electrode 14. Then, the face plate 15 is attached through an indium seal 16 to the opening of the envelope 10 to close it, thereby sealing the target 7 in the envelope 10.

The envelope 10 accommodating these members is heated at a temperature of about 120°C for vacuum evacuation to complete a vidicon. When an aluminum

55 As apparent from Table 1 above, a semi-insulating layer of Sb<sub>2</sub>Se<sub>3</sub> or Sb<sub>2</sub>S<sub>3</sub>, when treated at higher temperatures than about 250°C, substantially failed to be put to practical use, whereas a semi-insulating layer made of cadmium compounds, when treated even at 400°C, only slightly varied in resistance and was not solidified or revolatilized, proving that heat treatment at such level of temperature did not harmfully affect its performance.

60 Referring to Table 1 above a temperature of 120°C is the level at which heat treatment is applied in the manufacture of a general vidicon. However, if heating is applied in evacuating a glass bulb at as high temperatures as it is not softened, it will expel the larger amounts of gas deposited on the inner bulb walls or electrodes placed therein, thereby improving the performance and life of a vidicon. Since it is desired to conduct evacua-

tion at as high a temperature as 400°C, a limit point at which the glass material is not softened, the target of the present invention offers great advantage because its properties are not deteriorated even by such high temperature treatment.

What we claim is:

1. A method for manufacturing an image pickup tube comprising steps of:

fabricating a semiconductor target including preparing a semiconductor substrate having one conductivity type, forming a plurality of island regions of the opposite conductivity type on one side of the substrate, forming an insulating layer on said one side of the substrate exclusive of the island regions thereof, and coating a semi-insulating layer of cadmium telluride at least on the insulating layer;

mounting said semiconductor target in a glass envelope; and then heating the envelope at a temperature of from 250° to 400°C for evacuation.

5 2. The method according to claim 1 comprising sealing the envelope with an aluminum seal after mounting of said target in said envelope and before heating of said envelope.

10 3. The method according to claim 1 further comprising mounting in the envelope an accelerating electrode, mesh electrode and electron gun.

15 4. The method according to claim 1 further comprising mounting in the envelope accelerating electrodes, a mesh electrode, an electron gun and a photosensitive surface.

\* \* \* \* \*

20

25

30

35

40

45

50

55

60

65